

E. WEINTRAUB & L. B. MILLER.

MICROPHONE.

APPLICATION FILED JAN. 31, 1914.

1,156,509.

Patented Oct. 12, 1915.

Fig. 1.



Fig. 2.



Witnesses:

J. Earl Ryan  
J. Ellis Elen

Inventors:  
Ezechiel Weintraub,  
Levi B. Miller,  
by *Alfred J. Dunn*,  
Their Attorney.

# UNITED STATES PATENT OFFICE.

EZECHIEL WEINTRAUB AND LEVI B. MILLER, OF LYNN, MASSACHUSETTS, ASSIGNORS  
TO GENERAL ELECTRIC COMPANY, A CORPORATION OF NEW YORK.

## MICROPHONE.

1,156,509.

Specification of Letters Patent.

Patented Oct. 12, 1915.

Application filed January 31, 1914. Serial No. 815,682.

*To all whom it may concern:*

Be it known that we, EZECHIEL WEINTRAUB and LEVI B. MILLER, citizens of the United States, residing at Lynn, in the county of Essex, State of Massachusetts, have invented certain new and useful Improvements in Microphones, of which the following is a specification.

The carbon microphone such as commonly used as a telephone transmitter increases in electrical resistance with continued use and its resistance eventually becomes so high as to make the microphone practically inoperative with a given working line voltage. This is especially true of those types of telephone apparatus in which the transmitter is held in hand by the user, and the microphone is assuming different positions whereby the powder is roughly shaken up.

We have discovered that when carbon having a hardness equal to or greater than 6 on the Mohs mineral scale is employed in a microphone that the resistance increases at a very much slower rate than with the softer carbon now used, so that the useful life of the microphone is lengthened. Other desirable properties of a telephone transmitter, such as clearness of enunciation, are also improved.

The accompanying drawings illustrate in Figure 1 a common form of telephone transmitter, and in Fig. 2 show in a more diagrammatic form a simple microphone which may be used for telephones or other purposes.

The hard carbon used in our improved microphone is preferably prepared from synthetic resins commonly known as condensation products, particularly the phenol-aldehyde resins, some of which are well-known by trade names, such as bakelite and condensite. Condensation products of a polyhydric alcohol, such, for example, as glycerin and a polybasic organic acid, for example, phthalic acid or its anhydrid may likewise be used. Good results are also obtained with carbon prepared from cellulose by methods similar to those employed in making the bases of ordinary carbon filaments used in incandescent lamps.

In order to prepare the carbon for use in the microphone, the resinous condensation products are heated first for about 20 to 30 hours to a temperature which continuously

rises from about 70° C. to about 290° C. 55 The heating may be carried on in an oven heated first by steam and then by gas combustion. This stage of the heating produces complete polymerization and hardening of the condensation products and drives out 60 gases. If it is desired to produce disks of this hard carbon such as indicated at 1 and 2 in the accompanying drawing, the resin should be shaped into disk form before heating, as shaping subsequent to hardening is 65 difficult, but if desired even the hardened resin may be machined into desired form. After the preliminary bake the hardened resin is carbonized. The resin is preferably packed in a carbon or graphite container in 70 a protective material, such, for example, as peat. The container, packed in coke, lamp-black, or the like, is slowly heated by gas combustion or electrically to a temperature rising to about 700° C. in about one week. 75 The carbon is given a final firing at a temperature rising from 800° to 1100° C. in a few hours. For the purpose of making carbon powder or granules such as shown at 3, Fig. 1, the carbon produced by this carbonizing treatment is pulverized and sized by sifting through screens of suitable mesh. The carbon disks are preferably plated on one side with copper, or other suitable metal. In a similar manner, buttons of hard carbon, 85 such as indicated at 4, may be used in conjunction with a carbon or metal plate 5.

The carbon is very bright and shiny looking and is hard enough to scratch ordinary soda-lime glass and has a conchoidal fracture. A large proportion of the carbon prepared as described above is hard enough to scratch quartz which on the Mohs scale has a hardness of about 7. Its conductivity may be varied by regulating the firing temperature, a higher firing temperature resulting in carbon of a greater conductivity. The granules of this very hard carbon can be used in the ordinary microphone transmitter instead of the softer carbon granules. A 90 standard form of transmitter such as shown in Fig. 1 may be used, comprising a frame 6 supporting a capsule 7 containing the carbon powder. The sound waves directed against a diaphragm 8 by a mouth-piece 9, 95 produce a varying pressure upon the carbon powder which is included in the electrical circuit.

In our opinion the increased life of the microphone is to be ascribed largely to the greater resistance to wear and to pulverizing action of impacts possessed by this hard carbon. In microphones formerly used some of the carbon appears to be converted into a fine dust which apparently is responsible for the increase of resistance.

To illustrate the improvement obtained in microphones by use of the hard form of carbon, the following results by actual tests may be described. The ordinary standard powder was used on a 48-volt circuit in one series of tests and carbon derived from the phenol-formaldehyde resin known as bakelite in another series. To make the tests severe the transmitter was shaken violently for a half hour by hitting it about once a second in different directions against a solid wall. After half an hour of such treatment the resistance of the standard powder went up from 150 ohms to 450 ohms, thus increasing in the ratio 3:1. The resistance of the microphone with the improved carbon increased from 100 ohms to 140 ohms, or only 40%. This would mean that the useful life of the microphone is increased five times by the employment of glass-hard carbon. Our new microphone also transmits speech with improved clearness or sharpness of enunciation.

What we claim as new and desire to secure by Letters Patent of the United States, is:—

1. A microphone having a member consisting of conductive carbon made by carbonizing a resinous condensation product, and having hardness at least about 6 on the Mohs scale. 35

2. A microphone containing granules consisting of conductive carbon made by carbonizing a resinous phenolic condensation product and being hard enough to scratch glass. 40

3. A microphone containing granules comprising conductive carbon having a hardness of at least about 6 on the Mohs scale, a shiny surface and a conchoidal fracture. 45

4. A microphone containing conductive granules of a carbonized resinous phenolic condensation product. 50

5. Conductive carbon granules, suitable for use in a microphone, having a hardness of at least about 6 on the Mohs scale, a shiny surface and a conchoidal fracture.

In witness whereof, we have hereunto set our hands this 28th day of January, 1914. 55

EZECHIEL WEINTRAUB.  
LEVI B. MILLER.

Witnesses:

JOHN A. McMANUS, Jr.,  
HENRY A. ANDERSEN.

Copies of this patent may be obtained for five cents each, by addressing the "Commissioner of Patents.  
Washington, D. C."